

**1**

2,825,647

**PHOTOGRAPHIC DEVELOPER**

Robert E. Fuller, Woburn, Mass.

 No Drawing. Application October 28, 1954  
 Serial No. 465,450

7 Claims. (Cl. 96—66)

This invention relates to photography, and more particularly to photographic developers of improved and advantageous characteristics.

By the present invention, there is provided an all-purpose photographic developer capable of producing negatives and prints of fine photographic quality, and yet which exhibits characteristics affording great convenience in storage and use. Photographically, among other qualities, the developer exhibits the unique combination of properties of developing rapidly and yet producing negatives and prints of very fine grain. The developer exhibits good keeping qualities, both before and after solution in water. A marked advantage for the amateur is that the developer may be made in the form of a one-part developer, either powder or tablet, and a highly advantageous feature is that the developer may be prepared in the form of a readily soluble, effervescent powder or tablet.

The developer of this invention is characterized by the presence of sizable proportions of sodium acetate therein, for example, from about 20% to about 60% by weight of the dry solids of the developer. The pH of the developer in aqueous solution may range from about 8 to about 11, and a pH of 9 has been found highly suitable. When the developer is prepared as an effervescent powder or tablet, the sodium acetate may be incorporated in whole or in part in the form of sodium diacetate, the formula of which may be given as



The sodium diacetate also provides a source of acid in dry form for the developer prepared as an effervescent powder or tablet.

The developer of this invention contains other constituents conventional in developers in general. The nature of the reducing agent, or silver halide developer, is not critical, but it has been found that the use of Metol (p-methylaminophenol sulfate) and hydroquinone in combination is very effective, although the invention is not limited thereto. A preservative for the developer is preferably present, such as the commonly employed sodium sulfite. An accelerator of the developer such as sodium carbonate is usually incorporated. The sodium carbonate also provides a source of carbon dioxide for the effervescent powder or tablet. Ordinarily the use of a restrainer of the developer such as potassium bromide is not necessary, although its use is not precluded. Other types of constituents may be incorporated if desired.

The invention may be illustrated by a developer in the form of an effervescent tablet wherein the total sodium acetate content is derived from the sodium diacetate and

**2**

a portion of the sodium carbonate incorporated therein. The composition of such developer is as follows:

**Example 1**

|    |                                                                       | Ounces avoirdupois |
|----|-----------------------------------------------------------------------|--------------------|
| 5  | Metol (p-methylaminophenol sulfate)                                   | 4.8                |
|    | Hydroquinone                                                          | 6.1                |
|    | Anhydrous sodium sulfite                                              | 30.                |
|    | Sugar                                                                 | 3.                 |
| 10 | Sodium carbonate monohydrate                                          | 40.4               |
|    | Anhydrous sodium diacetate (containing approximately 40% acetic acid) | 26.4               |
|    | <b>Total</b>                                                          | <b>110.7</b>       |

15 In the above composition the Metol and hydroquinone are reducing agents or the silver halide developer, the sodium sulfite is a preservative for the developer, and the sugar is a binder or tabletting agent. The sodium carbonate is an accelerator of the developer, and when the tablet is dissolved in water, a portion of the sodium carbonate reacts with the acetic acid content of the sodium diacetate to impart effervescence, as well as to form additional sodium acetate in solution. In the above composition the available sodium acetate present is slightly over 27½% by weight of the solids.

20 The tablet of this example may be prepared by compounding the Metol, hydroquinone and sodium sulfite thoroughly, and then adding the sugar together with 3 fluid ounces of water, and beating the mixture to produce a moist conglomerate. The conglomerate is then dried, for example, by heating for about 45 minutes on coils containing steam at 6 lbs. pressure. The resulting dried material is then ground to about 14–16 mesh, to produce a granular material suitable for tablet making.

25 The sodium diacetate and sodium carbonate are then mixed with the granular material described in the preceding paragraph. The mixture is thoroughly drummed, for example for about 30 minutes, and then pressed into tablets. Conveniently the tablets may weigh 75 grains each.

30 To form a developing solution, one 75-grain tablet may be dissolved in 8 fluid ounces of water, and the resulting solution exhibits a pH of about 9. Due to the effervescent character of the tablet, the solution thereof takes place readily. At this concentration, ordinary film may be developed in 5 minutes at 68° F.

35 In Example 2, given below, there is illustrated an effervescent tablet, similar to that of Example 1, except that a mixture of sodium acetate and sodium diacetate is employed to provide the available sodium acetate content.

**Example 2**

|    |                                                                       | Ounces avoirdupois |
|----|-----------------------------------------------------------------------|--------------------|
| 55 | Metol                                                                 | 4.8                |
|    | Hydroquinone                                                          | 6.1                |
|    | Anhydrous sodium sulfite                                              | 30.                |
|    | Sugar                                                                 | 3.                 |
| 60 | Sodium carbonate monohydrate                                          | 33.8               |
|    | Anhydrous sodium diacetate (containing approximately 40% acetic acid) | 19.8               |
|    | Anhydrous sodium acetate                                              | 11.                |
|    | <b>Total</b>                                                          | <b>108.5</b>       |

In the above composition, the constituents have the

same functions as described in connection with Example 1. The sodium acetate content is provided only in part by sodium diacetate and the remainder is provided by sodium acetate added as such. Less sodium carbonate is employed than in the case of Example 1. In Example 2, the available sodium acetate is slightly over 31% by weight of the solids.

The effervescent tablet of Example 2 may be prepared in the same manner as that of Example 1, the sodium acetate being added with the sodium diacetate and sodium carbonate. Again, the resulting tablets may weigh 75 grains each.

As in Example 1, one 75-grain tablet dissolves readily in 8 ounces of water to form a developing solution exhibiting a pH of about 9. Ordinarily film develops therein in 5 minutes at 68° F.

Example 3, given below, illustrates a one-part developer according to this invention, in the form of an effervescent powder.

*Example 3*

|                                                                       | Ounces avoirdupois |
|-----------------------------------------------------------------------|--------------------|
| Metol (p-methylaminophenol sulfate)                                   | 4.8                |
| Hydroquinone                                                          | 6.1                |
| Anhydrous sodium sulfite                                              | 30.                |
| Sugar                                                                 | 3.                 |
| Sodium carbonate monohydrate                                          | 40.4               |
| Anhydrous sodium diacetate (containing approximately 40% acetic acid) | 26.4               |
| Total                                                                 | 110.7              |

The above composition of Example 3 is identical with that of Example 1. The compounding procedure is the same as set forth under Example 1 except that the tabletting step is omitted. The resulting product is an effervescent powder.

To form a developing solution, 75 grains of the effervescent powder may be dissolved in 8 fluid ounces of water. The resulting solution exhibits a pH of about 9, and ordinary film may be developed therein in 5 minutes at 68° F.

Example 4, given below, illustrates another one-part developer according to the invention, which in this case is in the form of a non-effervescent powder.

*Example 4*

|                                     | Ounces avoirdupois |
|-------------------------------------|--------------------|
| Metol (p-methylaminophenol sulfate) | 2.0                |
| Hydroquinone                        | 2.5                |
| Anhydrous sodium sulfite            | 30.0               |
| Sodium carbonate monohydrate        | 12.0               |
| Anhydrous sodium acetate            | 45.0               |
| Total                               | 91.5               |

The composition of this example, which contains slightly over 49% by weight of sodium acetate, may be prepared by mixing together the Metol, hydroquinone and sodium sulfite, and then adding the sodium carbonate and sodium acetate, followed by thorough mixing of the entire composition.

To form a developing solution, 125 grains of the above powder may be dissolved in 8 fluid ounces of water, the resulting solution exhibiting a pH of about 9. At this concentration, ordinary film may be developed in 5 minutes at 68° F.

For the developing of prints, the concentrations of the aqueous solutions may be somewhat greater than given above. Thus, for print development, the amounts of solid developer set forth in the specific examples may be dissolved in 6 fluid ounces of water.

By the present invention, there is provided an all-purpose developer, capable of producing film negatives and prints of superior quality.

An outstanding characteristic of the developer is its capability of developing at high speed, while producing

negatives of very fine grain. By way of illustration, developers in accordance with the above examples have been used to develop Eastman Super XX 35 mm. film in 5 minutes with extremely fine grain, whereas other fine grain developers require from 16 to 30 minutes to produce equivalent results.

Developers of this invention exhibit further features of photographic excellence, such as the production of excellent shadow detail, and the exhibition of high resolving power.

Developing compositions according to the present invention are highly advantageous in use. In the powder or tablet form, they exhibit excellent keeping qualities, and present the advantage of a one-part developer, which may be used for the convenient preparation of small quantities of developing solution. In solution form, the developers also exhibit good keeping qualities. In general, the developer presents the feature of economy.

The developer of this invention may be utilized advantageously as a one-part developer, in the form of effervescent tablets, effervescent powder, or non-effervescent powder. Ordinarily there is no advantage in preparing the developer in the form of a non-effervescent tablet. Certain advantages of the invention may be obtained by preparing the composition as a multi-part developer.

It will be understood that variations in the composition of the developer may be made while still coming within the scope of the invention. Thus, various reducing agents, preservatives and other developer constituents may be employed. The source of sodium acetate may be varied; for example, sodium diacetate containing 34% acetic acid may be utilized, alone, or in admixture with sodium acetate.

The time of development may also be varied within the scope of the invention. This may be accomplished by varying the formulation with respect to accelerator or otherwise, or by varying other factors, such as concentration or temperature of solution.

The time of development may also be varied within the scope of the invention. This may be accomplished by varying the formulation with respect to accelerator or otherwise, or by varying other factors, such as concentration or temperature of solution.

The invention advantageously may be employed in color photography as well as in black-and-white photography, and may be utilized in the development of prints as well as of negatives.

It will be understood that various changes may be made without departing from the invention as herein disclosed.

Having described my invention, what I claim as new and desire to secure by Letters Patent of the United States is:

1. A photographic developing bath comprising, in aqueous solution, a silver halide developer, a preservative, sodium carbonate, and sodium acetate in amount from about 20% to about 60% by weight of the solids in said solution, said sodium carbonate being present in sufficient amount to impart to said bath a pH of from about 8 to about 11.

2. A solid photographic developing composition soluble in water to produce a developing bath, said composition comprising a silver halide developer, a preservative, sodium carbonate, and sodium acetate in amount from about 20% to about 60% by weight of said solid composition, said sodium carbonate being present in sufficient amount to impart a pH of from about 8 to about 11 to an aqueous developing bath prepared from said composition.

3. A solid photographic developing composition soluble in water to produce a developing bath, said composition comprising p-methylaminophenol sulfate, hydroquinone, sodium sulfite, sodium carbonate, and sodium acetate in amount from about 20% to about 60% by weight of said solid composition, said sodium carbonate being pres-

ent in sufficient amount to impart a pH of from about 8 to about 11 to an aqueous photographic developing bath prepared from said composition.

4. A solid, water-soluble, effervescent, photographic developing composition comprising a silver halide developer, a preservative, sodium carbonate, and sodium diacetate sufficient to provide available sodium acetate in amount from about 20% to about 60% by weight of said composition, said sodium carbonate being present in sufficient amount to produce sodium acetate in solution from the acetic acid content of said sodium diacetate and to impart a pH of from about 8 to about 11 to an aqueous photographic developing bath prepared from said composition.

5. A solid, water-soluble, effervescent, photographic developing composition comprising a silver halide developer, a preservative, sodium carbonate, and sodium acetate and sodium diacetate together sufficient to provide available sodium acetate in amount from about 20% to about 60% by weight of said composition, said sodium carbonate being present in sufficient amount to produce sodium acetate in solution from the acetic acid content of said sodium diacetate and to impart a pH of from about 8 to about 11 to an aqueous photographic developing bath prepared from said composition.

6. A solid, water-soluble, effervescent, photographic developing composition in the form of a tablet, said tablet comprising a silver halide developer, a preservative, sodium carbonate, and material including sodium diacetate

sufficient to provide available sodium acetate in amount from about 20% to about 60% by weight of said tablet, said sodium carbonate being present in sufficient amount to produce sodium acetate in solution from the acetic acid content of said sodium diacetate and to impart a pH of from about 8 to about 11 to an aqueous photographic developing bath prepared from said composition.

7. A solid, water-soluble, effervescent, photographic developing composition in the form of a tablet, said tablet containing p-methylaminophenol sulfate, hydroquinone, sodium sulfite, sodium carbonate, and sodium diacetate sufficient to provide available sodium acetate in amount from about 20% to about 60% by weight of said tablet, said sodium carbonate being present in sufficient amount to produce sodium acetate in solution from the acetic acid content of said sodium diacetate and to impart a pH of from about 8 to about 11 to an aqueous photographic developing bath prepared from said composition.

20 References Cited in the file of this patent  
UNITED STATES PATENTS

|           |          |               |
|-----------|----------|---------------|
| 1,158,011 | Thatcher | Oct. 26, 1915 |
| 1,990,800 | Russell  | Feb. 12, 1935 |
| 2,091,689 | Russell  | Aug. 31, 1937 |
| 2,606,118 | Rogers   | Aug. 5, 1952  |

25 FOREIGN PATENTS  
311,546 Great Britain May 16, 1929